

## 1

3,131,630

### PLANOGRAPHIC PRINTING PLATES

Alexander Spencer, Kingsbury, London, England, assignor to Gestetner Limited, London, England, a British company

No Drawing. Filed June 3, 1960, Ser. No. 33,629  
Claims priority, application Great Britain June 8, 1959  
14 Claims. (Cl. 101—149.2)

This invention relates to planographic printing plates. In recent years there have been developed various forms of so-called planographic printing plates which are effectively lithographic plates in which the image and non-image areas of the plate are distinguished in that the former is oleophilic and therefore receptive to greasy printing ink and the latter is hydrophilic and therefore rejects such ink. These plates are imaged either directly, for example by applying a greasy ink receptive image to the surface of the plate or may be pre-sensitized and the image produced by photographic or related means.

Basically therefore the plates must have a surface layer which can readily be rendered differentially ink-receptive and ink-repellent. The base material of the plates may be metal, e.g. thin aluminium sheet, but probably the bulk of the plates manufactured are on wet-strength paper base. Many proposals have been made for the precise structure of the plates, including the provision of waterproofing layers for the paper, anti-curl coatings and the like.

The surface coating, which is to accept the image, is referred to as the planographic coating or layer and normally consists of a colloid film-forming material. This must be essentially hydrophilic but must be insolubilised. Suitable colloids which have been proposed are carboxymethylcellulose, polyvinyl alcohol and polyacrylic resins.

It has been proposed to render such colloid layers insoluble by the application of salts of multivalent metals, e.g. copper and zinc, applied as a wash to the surface of the coated plate. This however involves a separate insolubilisation step and it is more convenient to include in the planographic coating a material which, when the coating is dried, will automatically insolubilise it. Proposals of this type which have been made in the past however have presented considerable difficulty since it is necessary that the insolubilising agent should not become effective before the coating is applied to the base sheet (or the coating solution becomes unusable) and that it should work rapidly and completely when the coating is dried (or else insolubilisation continues for a long period after the coating is made so that the degree of insolubilisation is difficult to fix and there are economic difficulties).

It is an object of the present invention to provide a new method for preparing a self-insolubilising colloid planographic coating for a planographic printing plate which avoids the difficulties referred to.

According to the present invention there is provided a process for the production of a planographic printing plate which comprises applying to a support sheet a layer of a coating composition comprising (a) a soluble complex formed of an acid-soluble hydrophilic colloid containing free hydroxy and/or carboxyl groups, one or more soluble multivalent metal salts and one or more volatile acids, and (b) a filler, the pH of the coating composition being below 7. Preferably, the composition further con-

## 2

tains a hardening agent for the hydrophilic colloid since in this way planographic printing plates may be obtained which will afford a larger number of copies before becoming unduly worn.

5 It is found that if there is added to a solution of an acid-soluble hydrophilic colloid, both a salt of a multivalent metal and a volatile acid, there is formed a soluble complex between the three which is quite stable at pH values below 7 but which when dried out decomposes rapidly to form an insoluble salt of the metal with the said colloid thus freeing the volatile acid which evaporates from the layer. The layer thus automatically insolubilises in situ. The composition advantageously also contains a hardening agent for the hydrophilic colloid in order that the layer should be given sufficient rigidity as a planographic printing layer that long runs of prints may be made from it, and the filler is included to give body to the layer and generally to render it more suitable for the acceptance of an image.

20 The support sheet may be of any suitable material such as metal, e.g. foil of aluminium or aluminium alloy, or paper, which may or may not have received a treatment to improve its wet-strength, or plastic foil. The support may carry sub-coated layers (i.e. layers between the support sheet and the planographic layer) e.g. waterproofing layers or layers serving to improve the anchorage of the planographic layer to the assembly.

25 Any acid-soluble hydrophilic colloid which contains free hydroxy and/or carboxyl groups may be used (such groups being necessary in order that the colloid should form salts with multivalent metals) and particularly satisfactory results have been obtained by the use of cellulose derivatives such as carboxymethyl cellulose, vinyl compounds such as vinyl acetates containing a proportion of free hydroxyl groups, and acrylic compounds such as polymeric acrylates and substituted acrylates.

30 The salt of a multivalent metal which is employed is in no way critical and any such soluble salt is suitable. Examples are the sulphates, nitrates, chlorides, acetates, formates and other soluble salts of copper, iron, nickel, cobalt and aluminium.

35 The selection of the acid is critical in the sense that it is essential that it should be volatile under the drying conditions applied to the coated plate. Generally this means that the acid should have a boiling point below about 150° C. Typical such acids are hydrochloric acid and the lower fatty acids, e.g. formic, acetic, propionic and butyric acids and the volatile substitution derivatives of such acids which still contain free carboxyl groups.

40 As already indicated it is advantageous to include in the planographic layer an agent which will have a hardening effect on the colloid which is formed by decomposition of the complex. The particular hardening agent of choice will depend on the colloid used and other factors but generally the most satisfactory results are obtained by using a chromate or bichromate as the hardening agent, e.g. alkali metal, ammonium, calcium or copper chromates or bichromates.

45 Any filler known for use in the art of planographic layers may be employed in the present invention. Generally a white pigment material is preferred, e.g. china clay, blanc fixe, zinc oxide, titanium dioxide or talc, but any other white pigment or a coloured pigment may be

employed. Of the commercially available fillers, china clay has been found to be most generally useful.

Due to the presence of the free volatile acid the coating composition has a pH value below 7 and generally it is preferred that it should be so formulated that it has a pH value below 5.

The coating compositions as aforesaid are conveniently applied by air-knife coating or brush coating, the coating weight being selected to suit the particular product being manufactured and generally being within the range of 2 to 10 lbs. per ream (calculated as dried-down coating). The ream referred to is a ream of 500 sheet 20 inches x 30 inches.

The following examples in which all the parts are by weight will serve to illustrate the invention:

#### EXAMPLE I

##### A. Preparation of a Paper-Base Support

Wet strength paper (45 lb. per ream) is given a back coating to ensure that the final product does not curl. A typical formulation is as follows:

| A              |    | Parts |
|----------------|----|-------|
| Casein         | 15 | 25    |
| Water          | 75 |       |
| Warm, then add |    |       |
| Ammonia        | 2  |       |
| B              |    | Parts |
| China clay     | 65 | 30    |
| Water          | 70 |       |

When the clay has been thoroughly dispersed, the dispersion is mixed with the casein solution and then the following made up solution is added.

| C                               |   | Parts |
|---------------------------------|---|-------|
| Zinc chloride solution 198° Tw. | 2 | 40    |
| Water                           | 5 |       |
| Ammonia                         | 5 |       |

This casein-china clay slurry is coated on the wire side of the wet strength paper in a coating weight of 2-8 lbs./ream.

The felt side of the wet strength paper is coated with an undercoating to ensure greater smoothness. A typical formulation is as follows:

| A              |    | Parts |
|----------------|----|-------|
| Casein         | 15 |       |
| Water          | 75 |       |
| Warm, then add |    |       |
| Ammonia        | 2  | 55    |

| B          |    | Parts |
|------------|----|-------|
| China clay | 65 | 60    |
| Water      | 70 |       |

This slurry is coated on to the felt side of the back-coated wet strength paper in a coating weight of 2-6 lbs./ream. The so-prepared base paper is ready for the planographic coating.

##### B. Application of the Planographic Coating

The following solutions were prepared:

| A                                             |     | Parts |
|-----------------------------------------------|-----|-------|
| Carboxy methyl cellulose solution:            |     |       |
| Low viscosity sodium carboxy methyl cellulose | 25  |       |
| Water (warm)                                  | 400 |       |
| Glacial acetic acid                           | 80  | 75    |

|                        |       |
|------------------------|-------|
| Clay slurry:           | Parts |
| China clay             | 100   |
| Water                  | 150   |
| 5 Salt Solution No. 1: | Parts |
| Copper sulphate        | 14    |
| Water                  | 50    |
| When dissolved add:    |       |
| Glacial acetic acid    | 4     |
| Salt Solution No. 2:   | Parts |
| Ammonium bichromate    | 8     |
| Water                  | 20    |
| Glacial acetic acid    | 2     |
| Salt Solution No. 3:   | Parts |
| Ferric chloride        | 3     |
| Water                  | 20    |
| Glacial acetic acid    | 10    |

A composite coating slurry was prepared from the above by mixing the clay slurry B with the carboxymethyl cellulose solution A and then simultaneously adding the Salt Solutions 1, 2 and 3. This slurry was coated on the undercoating of paper prepared as described above in coating weights between 2 to 10 lbs./ream.

#### EXAMPLE II

The following formulations were prepared:

| A                                  |       | Parts |
|------------------------------------|-------|-------|
| Medium viscosity polyvinyl alcohol | 25    |       |
| Water                              | 400   |       |
| Glacial acetic acid                | 80    |       |
| B                                  |       | Parts |
| China clay                         | 90    |       |
| Zinc oxide                         | 10    |       |
| Water                              | 150   |       |
| 40 Salt Solution No. 1:            | Parts |       |
| Copper sulphate                    | 14.0  |       |
| Water                              | 80.0  |       |
| Glacial acetic acid                | 12.0  |       |
| 45 Salt Solution No. 2:            | Parts |       |
| Ammonium bichromate                | 6     |       |
| Water                              | 30    |       |
| Glacial acetic acid                | 5     |       |

Compositions A and B were mixed and the salt solutions 1 and 2 added simultaneously. The resulting slurry was coated on the paper base described in Example IA at a coating weight of 2 to 10 lbs. per ream.

#### EXAMPLE III

The following formulations were prepared:

| A                                                  |       | Parts |
|----------------------------------------------------|-------|-------|
| Low viscosity carboxy methyl cellulose sodium salt | 25    |       |
| Water                                              | 400   |       |
| Glacial acetic acid                                | 80    |       |
| B                                                  |       | Parts |
| China clay                                         | 90    |       |
| Zinc oxide                                         | 10    |       |
| Water                                              | 150   |       |
| 65 Salt Solution No. 1:                            | Parts |       |
| Zinc chloride                                      | 14.0  |       |
| Water                                              | 80.0  |       |
| Glacial acetic acid                                | 12.0  |       |
| 70 Salt Solution No. 2:                            | Parts |       |
| Ammonium bichromate                                | 6     |       |
| Water                                              | 30    |       |
| Glacial acetic acid                                | 5     |       |

Formulations A and B were mixed and the salt solutions then added simultaneously. The resulting slurry was coated on paper base prepared as described in Example IA at a coating weight of 2 to 10 lbs. per ream.

## EXAMPLE IV

The following formulations were prepared:

A

|                                               | Parts |
|-----------------------------------------------|-------|
| Low viscosity sodium carboxy methyl cellulose | 25    |
| Water                                         | 400   |
| Glacial acetic acid                           | 80    |

B

|                 | Parts |
|-----------------|-------|
| China clay      | 90    |
| Barium sulphate | 10    |
| Water           | 150   |

|                      | Parts |
|----------------------|-------|
| Salt Solution No. 1: |       |
| Copper sulphate      | 14.0  |
| Water                | 80.0  |
| Glacial acetic acid  | 12.0  |
| Salt Solution No. 2: |       |
| Ammonium bichromate  | 6     |
| Water                | 30    |
| Glacial acetic acid  | 5     |

Formulations A and B were mixed and the salt solutions then added simultaneously. The resulting slurry was coated on paper base prepared as described in Example IA at a coating weight of 2 to 10 lbs. per ream.

## EXAMPLE V

The following formulations were prepared:

A

|                                               | Parts |
|-----------------------------------------------|-------|
| Low viscosity sodium carboxy methyl cellulose | 25    |
| Water                                         | 400   |
| Glacial acetic acid                           | 80    |

B

|                  | Parts |
|------------------|-------|
| China clay       | 90    |
| Titanium dioxide | 10    |
| Water            | 150   |

|                      | Parts |
|----------------------|-------|
| Salt Solution No. 1: |       |
| Copper sulphate      | 14.0  |
| Water                | 80.0  |
| Glacial acetic acid  | 12.0  |
| Salt Solution No. 2: |       |
| Ammonium bichromate  | 6     |
| Water                | 30    |
| Glacial acetic acid  | 5     |

Formulations A and B were mixed and the salt solutions then added simultaneously. The resulting slurry was coated on paper base prepared as described in Example IA at a coating weight of 2 to 10 lbs. per ream.

## EXAMPLE VI

The following formulations were prepared:

A

|                                               | Parts |
|-----------------------------------------------|-------|
| Low viscosity sodium carboxy methyl cellulose | 25    |
| Water                                         | 400   |
| Glacial acetic acid                           | 80    |

B

|            | Parts |
|------------|-------|
| China clay | 90    |
| Zinc oxide | 10    |
| Water      | 150   |

|                      | Parts |
|----------------------|-------|
| Salt Solution No. 1: |       |
| Nickel nitrate       | 14.0  |
| Water                | 80.0  |
| Glacial acetic acid  | 12.0  |
| Salt Solution No. 2: |       |
| Ammonium bichromate  | 6     |
| Water                | 30    |
| Glacial acetic acid  | 5     |

Formulations A and B were mixed and the salt solutions then added simultaneously. The resulting slurry was coated on paper base prepared as described in Example IA at a coating weight of 2 to 10 lbs. per ream.

## EXAMPLE VII

The following formulations were prepared:

A

|                                               | Parts |
|-----------------------------------------------|-------|
| Low viscosity sodium carboxy methyl cellulose | 25    |
| Water                                         | 400   |
| Glacial acetic acid                           | 80    |

B

|            | Parts |
|------------|-------|
| China clay | 90    |
| Zinc oxide | 10    |
| Water      | 150   |

|                      | Parts |
|----------------------|-------|
| Salt Solution No. 1: |       |
| Cobalt chloride      | 14.0  |
| Water                | 80.0  |
| Glacial acetic acid  | 12.0  |
| Salt Solution No. 2: |       |
| Ammonium bichromate  | 6     |
| Water                | 30    |
| Glacial acetic acid  | 5     |

Formulations A and B were mixed and the salt solutions then added simultaneously. The resulting slurry was coated on paper base prepared as described in Example IA at a coating weight of 2 to 10 lbs. per ream.

## EXAMPLE VIII

The following formulations were prepared:

A

|                                               | Parts |
|-----------------------------------------------|-------|
| Low viscosity sodium carboxy methyl cellulose | 25    |
| Water                                         | 400   |
| Glacial acetic acid                           | 80    |

B

|            | Parts |
|------------|-------|
| China clay | 90    |
| Zinc oxide | 10    |
| Water      | 150   |

|                      | Parts |
|----------------------|-------|
| Salt Solution No. 1: |       |
| Aluminium sulphate   | 14.0  |
| Water                | 80.0  |
| Glacial acetic acid  | 12.0  |
| Salt Solution No. 2: |       |
| Ammonium bichromate  | 6     |
| Water                | 30    |
| Glacial acetic acid  | 5     |

Formulations A and B were mixed and the salt solutions then added simultaneously. The resulting slurry was coated on paper base prepared as described in Example IA at a coating weight of 2 to 10 lbs. per ream.

## EXAMPLE IX

The following formulations were prepared:

A

|                                               | Parts |
|-----------------------------------------------|-------|
| Low viscosity sodium carboxy methyl cellulose | 25    |
| Water                                         | 400   |
| Formic acid                                   | 80    |

7  
B

|            |     |
|------------|-----|
| Parts      |     |
| China clay | 90  |
| Zinc oxide | 10  |
| Water      | 150 |

|                      |      |
|----------------------|------|
| Parts                |      |
| Salt Solution No. 1: |      |
| Copper sulphate      | 14.0 |
| Water                | 80.0 |
| Formic acid          | 12.0 |

|                      |    |
|----------------------|----|
| Parts                |    |
| Salt Solution No. 2: |    |
| Ammonium bichromate  | 6  |
| Water                | 30 |
| Formic acid          | 5  |

|                      |      |
|----------------------|------|
| Parts                |      |
| Salt Solution No. 3: |      |
| Ferric chloride      | 3.2  |
| Water                | 20.0 |
| Formic acid          | 10.0 |

Formulations A and B were mixed and the salt solutions then added simultaneously. The resulting slurry was coated on paper base prepared as described in Example IA at a coating weight of 2 to 10 lbs. per ream.

## EXAMPLE X

The following formulations were prepared:

A

|                                               |     |
|-----------------------------------------------|-----|
| Parts                                         |     |
| Low viscosity sodium carboxy methyl cellulose | 25  |
| Water                                         | 400 |
| Butyric acid                                  | 80  |

B

|            |     |
|------------|-----|
| Parts      |     |
| China clay | 90  |
| Zinc oxide | 10  |
| Water      | 150 |

|                      |      |
|----------------------|------|
| Parts                |      |
| Salt Solution No. 1: |      |
| Copper sulphate      | 14.0 |
| Water                | 80.0 |
| Butyric acid         | 12.0 |

|                      |    |
|----------------------|----|
| Parts                |    |
| Salt Solution No. 2: |    |
| Ammonium bichromate  | 6  |
| Water                | 30 |
| Butyric acid         | 5  |

Formulations A and B were mixed and the salt solutions then added simultaneously. The resulting slurry was coated on paper base prepared as described in Example IA at a coating weight of 2 to 10 lbs. per ream.

## EXAMPLE XI

The following formulations were prepared:

A

|                                               |     |
|-----------------------------------------------|-----|
| Parts                                         |     |
| Low viscosity sodium carboxy methyl cellulose | 25  |
| Water                                         | 400 |
| Hydrochloric acid                             | 80  |

B

|            |     |
|------------|-----|
| Parts      |     |
| China clay | 90  |
| Zinc oxide | 10  |
| Water      | 150 |

|                      |      |
|----------------------|------|
| Parts                |      |
| Salt Solution No. 1: |      |
| Copper sulphate      | 14.0 |
| Water                | 80.0 |
| Hydrochloric acid    | 12.0 |

|                      |    |
|----------------------|----|
| Parts                |    |
| Salt Solution No. 2: |    |
| Ammonium bichromate  | 6  |
| Water                | 30 |
| Hydrochloric acid    | 5  |

Formulations A and B were mixed and the salt solutions then added simultaneously. The resulting slurry was

coated on paper base prepared as described in Example IA at a coating weight of 2 to 10 lbs. per ream.

8

The following formulations were prepared:

A

|                                               |     |
|-----------------------------------------------|-----|
| Parts                                         |     |
| Low viscosity sodium carboxy methyl cellulose | 25  |
| Water                                         | 400 |
| 10 Acetic acid                                | 80  |

B

|            |     |
|------------|-----|
| Parts      |     |
| China clay | 90  |
| Zinc oxide | 10  |
| Water      | 150 |

|                      |      |
|----------------------|------|
| Parts                |      |
| Salt Solution No. 1: |      |
| Copper chromate      | 14.0 |
| Water                | 250  |
| Acetic acid          | 250  |

|                      |    |
|----------------------|----|
| Parts                |    |
| Salt Solution No. 2: |    |
| Ammonium bichromate  | 6  |
| Water                | 30 |
| Acetic acid          | 5  |

Formulations A and B were mixed and the salt solutions then added simultaneously. The resulting slurry was coated on paper base prepared as described in Example IA at a coating weight of 2 to 10 lbs. per ream.

## EXAMPLE XIII

The following formulations were prepared:

A

|                     |     |
|---------------------|-----|
| Parts               |     |
| Sodium polyacrylate | 25  |
| Water               | 400 |
| Acetic acid         | 80  |

B

|            |     |
|------------|-----|
| Parts      |     |
| China clay | 90  |
| Zinc oxide | 10  |
| Water      | 150 |

|                      |      |
|----------------------|------|
| Parts                |      |
| Salt Solution No. 1: |      |
| Nickel nitrate       | 14.0 |
| Water                | 80.0 |
| Acetic acid          | 12.0 |

|                      |    |
|----------------------|----|
| Parts                |    |
| Salt Solution No. 2: |    |
| Ammonium bichromate  | 6  |
| Water                | 30 |
| Acetic acid          | 5  |

Formulations A and B were mixed and the salt solutions then added simultaneously. The resulting slurry was coated on paper base prepared as described in Example IA at a coating weight of 2 to 10 lbs. per ream.

## EXAMPLE XIV

The following formulations were prepared:

A

|                                              |     |
|----------------------------------------------|-----|
| Parts                                        |     |
| Low viscosity sodium carboxymethyl cellulose | 25  |
| Water                                        | 400 |
| Glacial Acetic Acid                          | 80  |

B

|            |     |
|------------|-----|
| Parts      |     |
| China clay | 90  |
| Zinc oxide | 10  |
| Water      | 150 |

|                      |      |
|----------------------|------|
| Parts                |      |
| Salt Solution No. 1: |      |
| Nickel nitrate       | 14.0 |
| Water                | 80.0 |
| Acetic acid          | 12.0 |

Formulations A and B were mixed and the salt solutions then added simultaneously. The resulting slurry was

75

|                      |       |
|----------------------|-------|
| Salt Solution No. 2: | Parts |
| Ammonium bichromate  | 6     |
| Water                | 30    |
| Glacial Acetic acid  | 5     |
| Salt Solution No. 3: | Parts |
| Ferric chloride      | 3.0   |
| Water                | 20.0  |
| Formic acid          | 10.0  |

Formulations A and B were mixed and the salt solutions then added simultaneously. The resulting slurry was coated on paper base prepared as described in Example IA at a coating weight of 2 to 10 lbs. per ream.

## EXAMPLE XV

The following formulations were prepared:

## A

|                                               |       |
|-----------------------------------------------|-------|
| Low viscosity sodium carboxy methyl cellulose | Parts |
| Water                                         | 25    |
| Glacial acetic acid                           | 20    |

## B

|                      |       |
|----------------------|-------|
| China clay           | Parts |
| Zinc oxide           | 90    |
| Water                | 10    |
|                      | 150   |
| Salt Solution No. 1: | Parts |
| Zinc chloride        | 8.0   |
| Water                | 40.0  |
| Acetic acid          | 8.0   |
| Salt Solution No. 2: | Parts |
| Nickel sulphate      | 8.0   |
| Water                | 40.0  |
| Acetic acid          | 8.0   |
| Salt Solution No. 3: | Parts |
| Copper chromate      | 8     |
| Water                | 160   |
| Acetic acid          | 160   |

Formulations A and B were mixed and the salt solutions then added simultaneously. The resulting slurry was coated on paper base prepared as described in Example IA at a coating weight of 2 to 10 lbs. per ream.

## EXAMPLE XVI

The following formulations were prepared:

## A

|                                               |       |
|-----------------------------------------------|-------|
| Low viscosity sodium carboxy methyl cellulose | Parts |
| Water                                         | 25    |
| Glacial Acetic acid                           | 400   |

## B

|                      |       |
|----------------------|-------|
| China clay           | Parts |
| Zinc oxide           | 90    |
| Water                | 10    |
|                      | 150   |
| Salt Solution No. 1: | Parts |
| Copper sulphate      | 14    |
| Water                | 80    |
| Acetic acid          | 12    |
| Salt Solution No. 2: | Parts |
| Calcium chromate     | 6.0   |
| Water                | 12.0  |
| Acetic acid          | 1.0   |

Formulations A and B were mixed and the salt solutions then added simultaneously. The resulting slurry was coated on paper base prepared as described in Example IA at a coating weight of 2 to 10 lbs. per ream.

## EXAMPLE XVII

The following formulations were prepared:

## A

|                                               |       |
|-----------------------------------------------|-------|
| 5                                             | Parts |
| Low viscosity sodium carboxy methyl cellulose | 25    |
| Water                                         | 400   |
| Glacial acetic acid                           | 80    |

## 10

|            |
|------------|
| Parts      |
| China clay |
| Zinc oxide |
| Water      |

## 15

|                     |
|---------------------|
| Parts               |
| Copper sulphate     |
| Water               |
| Glacial acetic acid |

|                     |
|---------------------|
| Parts               |
| Zinc chloride       |
| Water               |
| Glacial acetic acid |

Formulations A and B were mixed and the salt solutions then added simultaneously. The resulting slurry was coated on paper base prepared as described in Example IA in a coating weight of 2 to 10 lbs. per ream. Since the composition in this case contains no hardening agent for the hydrophilic colloid, the resulting plate effects a lesser number of satisfactory prints before becoming too damaged.

Whilst in all the foregoing examples the coating composition is directed to be applied to a paper base prepared as in Example IA it is to be understood that the coatings may be applied to paper base without an intervening undercoating. The undercoating is generally preferred however as it tends to smooth out roughnesses in the support sheet and it may also serve to increase the anchorage of the layers of the product. It is further to be understood that the coating weights of the planographic layer and the underlayers present may be varied as required.

To facilitate the production of flat, non-curling sheets, the various coatings may be submitted to calendering after application.

It has been found that by means of the present invention planographic plates may be produced in which the planographic coating becomes insolubilised and reaches a state of equilibrium in a short period, e.g. only a few days, and that the resulting plates are capable of yielding greater numbers of copies than plates similarly prepared but in which other methods of insolubilisation have been employed.

I claim:

1. A process for the production of a planographic printing plate which comprises applying to a support sheet a layer of a coating composition comprising (a) a soluble complex formed of an acid-soluble hydrophilic colloid, at least one multivalent metal salt and at least one volatile lower fatty acid, (b) a filler, and (c) a hardening agent for the hydrophilic colloid, the pH of the composition being below 7.

2. A process for the production of a planographic printing plate which comprises applying to a support sheet a layer of a coating composition comprising (a) a soluble complex formed of an acid-soluble hydrophilic colloid which is a soluble salt of carboxymethyl cellulose, at least one multivalent metal salt and at least one volatile lower fatty acid, (b) a filler, and (c) a hardening agent for the hydrophilic colloid, the pH of the composition being below 7.

3. A process for the production of a planographic printing plate which comprises applying to a support sheet a layer of a coating composition comprising (a) a soluble complex formed of an acid-soluble hydrophilic

## 11

colloid which is a polyvinyl alcohol, at least one multivalent metal salt and at least one volatile lower fatty acid, (b) a filler, and (c) a hardening agent for the hydrophilic colloid, the pH of the composition being below 7.

4. A process for the production of a planographic printing plate which comprises applying to a support sheet a layer of a coating composition comprising (a) a soluble complex formed of an acid-soluble hydrophilic colloid which is a soluble polyacrylate salt, at least one multivalent metal salt and at least one volatile lower fatty acid, (b) a filler, and (c) a hardening agent for the hydrophilic colloid, the pH of the composition being below 7.

5. A process for the production of a planographic printing plate which comprises applying to a support sheet a layer of a coating composition comprising (a) a soluble complex formed of an acid-soluble hydrophilic colloid, at least one multivalent metal salt selected from the class consisting of soluble sulphates, nitrates, chlorides, acetates and formates of copper, iron, nickel, cobalt and aluminium and at least one volatile lower fatty acid, (b) a filler, and (c) a hardening agent for the hydrophilic colloid, the pH of the composition being below 7.

6. A process for the production of a planographic printing plate which comprises applying to a support sheet a layer of a coating composition comprising (a) a soluble complex formed of an acid-soluble hydrophilic colloid which is a soluble salt of carboxymethyl cellulose, at least one multivalent metal salt selected from the class consisting of soluble sulphates, nitrates, chlorides, acetates and formates of copper, iron, nickel, cobalt and aluminium and at least one volatile lower fatty acid, (b) a filler, and (c) a hardening agent for the hydrophilic colloid, the pH of the composition being below 7.

7. A process for the production of a planographic printing plate which comprises applying to a support sheet a layer of a coating composition comprising (a) a soluble complex formed of an acid-soluble hydrophilic colloid, at least one multivalent metal salt and acetic acid, (b) a filler, and (c) a hardening agent for the hydrophilic colloid, the pH of the composition being below 7.

8. A process for the production of a planographic printing plate which comprises applying to a support sheet a layer of a coating composition comprising (a) a soluble complex formed of an acid-soluble hydrophilic colloid, at least one multivalent metal salt and formic acid, (b) a filler, and (c) a hardening agent for the hydrophilic colloid, the pH of the composition being below 7.

9. A process for the production of a planographic printing plate which comprises applying to a support sheet a layer of a coating composition comprising (a) a soluble complex formed of an acid-soluble hydrophilic colloid, which is a soluble salt of carboxymethyl cellulose, at least one multivalent metal salt selected from the class consisting of soluble sulphates, nitrates, chlorides, acetates and formates of copper, iron, nickel, cobalt and aluminium, and acetic acid, (b) a filler, and (c) a hardening agent for the hydrophilic colloid, the pH of the composition being below 7.

## 12

10. A process for the production of a planographic printing plate which comprises applying to a support sheet a layer of a coating composition comprising (a) a soluble complex formed of an acid-soluble hydrophilic colloid, at least one multivalent metal salt and at least one volatile acid, (b) a filler, and (c) a chromate hardening agent for the hydrophilic colloid, the pH of the composition being below 7.

11. A process for the production of a planographic printing plate which comprises applying to a support sheet a layer of a coating composition comprising (a) a soluble complex formed of an acid-soluble hydrophilic colloid which is a soluble salt of carboxymethyl cellulose, at least one multivalent metal salt and at least one volatile acid, (b) a filler, and (c) a chromate hardening agent for the hydrophilic colloid, the pH of the composition being below 7.

12. A process for the production of a planographic printing plate which comprises applying to a support sheet a layer of a coating composition comprising (a) a soluble complex formed of an acid-soluble hydrophilic colloid which is a soluble salt of carboxymethyl cellulose, at least one multivalent metal salt selected from the class consisting of soluble sulphates, nitrates, chlorides, acetates and formates of copper, iron, nickel, cobalt and aluminium and acetic acid, (b) a filler, and (c) a chromate hardening agent for the hydrophilic colloid, the pH of the composition being below 7.

13. A process for the production of a planographic printing plate which comprises applying to a support sheet a layer of a coating composition comprising (a) a soluble complex formed of an acid-soluble hydrophilic colloid, at least one multivalent metal salt and at least one volatile acid, (b), a filler containing china clay, and (c) a hardening agent for the hydrophilic colloid, the pH of the composition being below 7.

14. A process for the production of a planographic printing plate which comprises applying to a support sheet a layer of a coating composition comprising (a) a soluble complex formed of an acid-soluble hydrophilic colloid which is a soluble salt of carboxymethyl cellulose, at least one multivalent metal salt selected from the class consisting of soluble sulphates, nitrates, chlorides, acetates and formates of copper, iron, nickel, cobalt and aluminium and acetic acid, (b) a filler containing china clay, and (c) a chromate hardening agent for the hydrophilic colloid, the pH of the composition being below 7.

## References Cited in the file of this patent

## UNITED STATES PATENTS

|           |                      |               |
|-----------|----------------------|---------------|
| 2,230,981 | Toland et al. -----  | Feb. 4, 1941  |
| 2,534,650 | Worthen -----        | Dec. 19, 1950 |
| 2,542,784 | Van Dusen -----      | Feb. 20, 1951 |
| 2,550,326 | Brown -----          | Apr. 24, 1951 |
| 2,635,537 | Worthen -----        | Apr. 21, 1953 |
| 2,693,145 | Mullen -----         | Nov. 2, 1954  |
| 2,724,665 | Oransky et al. ----- | Nov. 22, 1955 |
| 2,808,778 | Newman et al. -----  | Oct. 8, 1957  |

## OTHER REFERENCES

Hercules Sodium Carboxymethylcellulose, Pub. 1944.